

Jan. 6, 1942.

C. R. BERNING

**2,269,355**

## MANUFACTURING OF ZINC OXIDE

Filed Sept. 26, 1936

2 Sheets-Sheet 1



Cornelius Raymond Keringer  
INVENTOR

BY *Mock & Blum*  
ATTORNEYS

Jan. 6, 1942.

C. R. BERINGER

2,269,355

MANUFACTURING OF ZINC OXIDE

Filed Sept. 26, 1936

2 Sheets-Sheet 2



Cornelius Raymond Beringer  
INVENTOR

BY *Mock & Blum*  
ATTORNEYS

## UNITED STATES PATENT OFFICE

2,269,355

## MANUFACTURING OF ZINC OXIDE

Cornelius Raymond Beringer, Pestszenterzsebet, Hungary, assignor, by mesne assignments, to Cornelius Raymond Beringer, Eugen Horvát, Ernst Horvát, Ferdinand Solt, and Alfred Spiegel, all of Budapest, Hungary

Application September 26, 1936, Serial No. 102,751  
In Germany September 28, 1935

3 Claims. (Cl. 23—148)

The invention relates to improvements in the manufacture of zinc oxide, particularly of zinc white, from metallic zinc, e. g. crude zinc, and/or from metals bearing zinc, e. g. lead bearing zinc, and/or from metal alloys bearing zinc, etc.

It is well known that in connection herewith difficulties result from the impurities, particularly from the lead contained in the metal bath to be evaporated because a portion of the impurities unavoidably passes into the zinc vapour atmosphere, and the said fact fundamentally impairs that best quality of product which from a given smelting bath is obtainable at all. On the other side, the portion of the impurities which does not pass over into the zinc vapour atmosphere will, in the course of the progress of manufacture, gradually (in proportion to the evaporation of the zinc) enrich the metal bath in regard to its contents of impurities, and in consequence thereof the percentage of impurities passing over into the zinc vapour atmosphere will also gradually increase.

The above facts result, altogether, in a fluctuation of the quality of the product obtained from one and the same metal bath. The difficulties as mentioned above considerably increase when initial materials of relative low purity are employed the use of which appears to be more advantageous owing to their lower price.

A number of proposals have already become known aiming at the diminution of the drawbacks referred to.

A former proposal of the inventor (see Austrian patent specification No. 105,794) is based on the fact that the portion of the impurities passing over into the zinc vapour atmosphere increases if the zinc is vaporised by means of an external heating imparted to the bottom of the bath because, in this case, the zinc bath may easily get into a condition of violent boiling and will show a tendency of forming bubbles. In view of the said fact, according to the above-mentioned earlier proposal of the inventor, the zinc bath is heated merely from above by radiated heat through effecting the combustion of the zinc vapours in a closed chamber above the zinc bath itself so that the zinc vapour layer produced above the bath burns down continuously from its upper side and is being continuously completed by supplementary surface evaporation at its under side. Although this process has the advantage that owing to the absence of any bottom heating there is nothing capable to prevent the separation of the impurities by eliquation in a depression provided in the zinc bath container,

the absence of any bottom heating, however, results in the possibility of heat being abstracted from the metal bath whereby the economy of this process may possibly become impaired.

5 In accordance with another earlier proposal (see German patent specification No. 444,863) the employment of relatively impure initial materials is rendered possible by inserting in series a special reverberatory furnace before the containers in which the molten zinc is converted from the fluid condition into the vapour condition, the said reverberatory furnace operating without any bottom heating in the manner of tub furnaces usually employed for refining crude zinc. Thereby the contents of impurities is being diminished in the said reverberatory furnace by means of eliquation to a degree low enough to be acceptable. This known process is extremely complicated and most expensive as regards working expenses and also as regards the first costs of the plant because the molten material prepared preliminarily in the reverberatory furnace for the purpose of purifying the zinc has to be conveyed from the said refining reverberatory furnace to 10 the other zinc bath containers and has to be poured over in order to enable the zinc to be converted there into vapour and to be oxidized subsequently.

In accordance with the present invention the 15 conversion of the zinc from the fluid condition into the vapour condition is effected in the same container in which the separation of the impurities by eliquation is also performed so that the drawbacks resulting from the preliminary smelting and pouring-over (as mentioned above) are wholly dispensed with and, on the other side, according to the invention, there is always provided a bottom heating too so that the drawback of abstracting heat from the melting bath, resulting in previous processes from the absence of bottom heating, is likewise wholly eliminated. According to the invention the above objects may be accomplished by performing the conversion of the molten material from the fluid condition into the vapour condition by means of bottom heating, or by means of bottom heating as well as by means of heating from above from a metal bath having a depressed extension which during the production of the zinc vapour at least partially, but preferably entirely, or in as great a degree as possible is exempted from the influence of said bottom heating.

Accordingly, the invention is based on the idea that separating the impurities by eliquation is possible also in case a bottom heating is em-

ployed and that it is possible to produce and maintain a very considerable temperature difference between various points of the bottom surface of the metal bath even in case the heating is carried to the point necessary to cause the molten zinc to become converted into vapour.

The removal of impurities by eliquation can be rendered more efficient by exposing the above-mentioned depressed extension of the metal bath to a cooling effect. I prefer to let the said cooling to act upon the said extension from all sides and, furthermore, I prefer to bring about the said cooling by means of air.

It is possible to carry the said cooling effect in the bottom part of the depression down to a temperature lying between the melting points of zinc and lead, respectively, so that the zinc is made to solidify in the lead etc. remaining still fluid in the bottom part of the depression whereby the zinc is enabled to float back again into the bath to those places which are exposed to the heating effect of said bottom heating. By these means it is possible to carry the separation of the impurities to a particularly high degree.

According to an exceedingly advantageous manner of carrying the process according to the invention into effect the metal bath is heated from above by means of radiated heat on its entire length whilst from the bottom it is heated along a portion of its length only and, at the same time, the non-heated part of the bottom of the metal bath is shaped to form a pocket-like depression.

The method preferably employed in connection herewith consists in heating the metal bath from above and also from its bottom by means of the heat of combustion of the zinc in such way that the said heat of combustion of the zinc acts upon the metal bath from above along its entire length and from the bottom but along a portion of its length. This may be accomplished in such way that the layer of zinc vapour produced above the bath is continuously being burned down from its upper side above the entire length of the metal bath itself and is, at the time, utilized to heat only a fraction of the walls of the evaporation chamber said heated walls of the evaporation chamber being brought at least partly (e. g. by the continuous or intermittent rotation of the melting kiln) underneath the metal bath and, at the same time, the said walls being shaped to form a pocket-like recess adapted to escape as far as possible the said heating effects of the heat of combustion of the zinc.

The utilisation of the heat of combustion of the zinc for providing a bottom heating by producing the metal bath in a rotary tube kiln is known (see for instance the German patent specification No. 557,499 of the inventor), and the provision of a depression within the said rotary tube kiln, for the purpose of depositing and collecting the impurities of greater specific weight, is also known. In the case of the said known process, however, the effect of the radiated heat acting upon the bath surface from above as well as the heating effect acting upon the bath from the bottom produced by the rotation of the kiln are both acting in the metal bath along its entire length because the depression provided inside the rotary tube kiln is always heated by the combustion of the zinc to the same temperature to which the other internal parts of the rotary tube kiln are heated. In fundamental contradistinction thereto according to the present invention differences of temperature are inten-

tionally produced at different parts of the bottom surface of the rotary tube kiln. Thereby the removal of the lead etc. by eliquation is rendered possible and the said removal is more independent of the casual circumstances of operation because, in the case of the process according to the present invention, both the difference of the specific weights of the various metals is utilized resulting in a separation merely by deposition as well as the difference of temperatures at different places of the bottom resulting in a separation of the various metals by eliquation too. As a result thereof the best quality of product obtainable from a melting bath having a certain degree of impurity is improved as compared to the known processes whilst, at the same time, the economy of operation is also increased and, moreover, operation is rendered more indifferent to any variations of the degree of purity of the melting bath which fact finds expression not only in the increased uniformity of the product obtained but also in the fact that the draining off of the impurities collected has to be effected at less frequent intervals.

With reference to the drawings which are of somewhat diagrammatic nature and for illustrative purposes only:

Fig. 1 is a side elevation in cross section and Fig. 2 is a cross-section through 2—2 of the rotary drum shown in Fig. 1; Figs. 3 and 4 are each illustrating a further embodiment of a melting drum according to the invention.

According to Figs. 1 and 2, the metal bath is produced in a rotary tube kiln *a* and the combustion of the zinc vapours is being effected within the said rotary tube kiln *a* itself, for which purpose air and/or other oxidizing gases (e. g. CO<sub>2</sub>) are introduced into the chamber *a*<sub>4</sub> of said kiln in such a manner that they pass over the layer of zinc vapour lying above the metal bath without coming into contact with the smelting-bath itself. Accordingly, the said layer will continuously burn down from above and will be continuously completed from underneath by the vapours coming from said metal bath whereby the surface of said metal bath is heated by radiation from above and the walls *a*<sub>1</sub>, *a*<sub>2</sub> of the rotary chamber *a*<sub>4</sub> are heated directly too.

For initiating the process a grate furnace *c* may be employed and the gases of combustion of said furnace may possibly also supply the CO<sub>2</sub>-containing gas in case such gas is employed for the combustion of the zinc in the chamber *a*<sub>4</sub>. It is preferably by rotating the kiln *a* that the heat of combustion of the zinc is utilized, in a manner per se known, for providing also a bottom heating. For this purpose the said kiln may be supported on rollers *k* as shown in such a manner that, by said rotating movement, the walls of the chamber *a*<sub>4</sub>, which are heated by the burning zinc vapours, get underneath the metal bath.

According to the invention the container for metal bath is shaped on its bottom to form a depressed extension *a*<sub>6</sub> constructed and arranged in such a manner that the bottom surface *a*<sub>7</sub> of said extension *a*<sub>6</sub> as well as its lateral walls should not be heated by the combustion taking place in the evaporation chamber *a*<sub>4</sub> or should be heated by the said combustion in a so small extent only that the said depressed extension *a*<sub>6</sub> is practically or in a so great extent as possible exempted from the effects of the bottom heating produced by rotating the kiln as explained above. Accordingly, the walls of the chamber *a*<sub>4</sub> and the molten metal contained in said chamber on the

one hand, and the walls of the extension  $a_6$  and the material contained in said extension on the other hand, possess different temperatures whereby, as has already been explained, the eliquation separating the impurities from the zinc is influenced in a most advantageous manner.

I prefer to separate the internal space of the depressed extension  $a_6$  from the internal space  $a_4$  of the drum  $a$  by one or a number of passages  $a_8$  whereby the maintenance of a lower temperature in the extension  $a_6$ , particularly at the bottom portion  $a_7$  of the latter as compared to the temperature of the bottom portion  $a_3$  is facilitated.

The internal space  $a_4$  of the drum  $a$  may be widened conically towards the extension  $a_6$  annularly surrounding the said drum so that the various metals capable of being separated by deposition and eliquation will tend to move towards the extension  $a_6$  already owing to their higher specific weight.

The depressed extension  $a_6$  forms an annular flange  $a_5$  around the drum  $a$  which flange is cooled on all sides by air whereby the temperature difference between the surfaces  $a_5$  and  $a_7$  is still further increased. In consequence of this temperature difference very substantial internal stresses are set up in the material of construction of said drum  $a$  so that it may become necessary to stiffen the said flange  $a_5$  in a suitable manner relatively to the shell surface of the drum  $a$  as indicated in Fig. 1.

The depressed extension  $a_6$  may be shaped according to any cross-sectional shape desired. I prefer to widen the said cross-section in the external direction, for instance in the manner of a truncated cone whereby the cooling effect within the range of the bottom surface  $a_7$  will still further increase.

By giving a suitable shape to the extension  $a_6$  and/or by employing suitable cooling agents, the cooling effect may be increased so far that in the extension  $a_6$  the zinc which possesses a higher melting-point will solidify and, accordingly, will rise in the lead etc. which still remains liquid thus returning again into the melting-bath located in the chamber  $a_4$ .

All impurities, valuable in themselves (lead, hard zinc etc.), collect in the extension  $a_6$  and may be removed, preferably each separately, through one or more closable openings provided on the side walls and/or bottom of said extension  $a_6$  as indicated in Fig. 1.

The rotation of the drum  $a$  may be effected by any desired means, e. g. by means of a preferably reversible electric motor  $r_4$ , through the gear parts  $r_2, r_3, r_1$ , or simply by means of rotating the rollers  $k$ , the drum  $a$  being then carried along by these rollers through friction.

According to Fig. 1, the zinc fumes stream from the chamber  $a_4$  into a duct  $g$  and hence, for the purpose of their being condensed to zinc white pigments, into a collecting device, etc. not shown. The supplementary feeding in of the zinc may be effected in any desired manner, e. g. through an opening  $h$  provided in the duct  $g$  and through the outlet opening  $f$  for the zinc fumes. Preferably, also air and/or some other oxidizing gas is introduced through the closable opening  $h$ , in order to cause a supplementary combustion of the zinc behind the outlet opening  $f$ . That part of the duct  $g$  which joins on to the rotary drum kiln  $a$  may be maintained at a high temperature to act as a storage chamber in which the zinc fumes may stay for some while.

According to Fig. 1, the flange  $a_5$  surrounding the depressed extension  $a_6$  of the smelting-bath is arranged at the outlet end of the drum  $a$ . In some cases it may be more advantageous to arrange the said flange  $a_5$  in accordance with Fig. 3 in the centre of the length of the drum and to widen the internal space  $a_4$  in diameter towards the middle of the length of the drum conically or in the shape of a barrel. Thereby, the length of the paths leading to the depression  $a_6$  are diminished as compared to the arrangement according to Fig. 1 and, thereby, the distribution of the internal stresses set up in the material of construction by the intentionally produced differences of temperature becomes also more favourable.

According to Fig. 4, depressed extensions  $a_6$  are provided in annular arrangement on both ends of the drum  $a$ , and the internal space is in this case widened from the middle of its length towards both ends.

Of course, more than two annular depressions  $a_6$  may be provided on the drum  $a$ , and it is also possible to provide outside the space  $a_4$  channels connecting the said depressions  $a_6$  with each other and establishing communication between them. Furthermore, it would also be possible to provide an annular extension  $a_6$  surrounding the drum  $a$  continuously following a helical or screw-like formation.

According to Fig. 1, the combustion of the zinc vapours is effected at least partly in the smelting chamber  $a_4$  above the zinc bath. If desired, however, the zinc vapours may be led out from said chamber  $a_4$  without combusting them therein. In this case the combustion will take place outside the chamber  $a_4$ , e. g. when the zinc vapours reach the duct  $g$ , and the bottom heating which extends but to a portion of the length of the smelting-bath must be effected by some other method known per se, for instance by electrical means. At the same time on the whole length of the smelting bath in any manner desired a non-oxidizing heating by means of radiated heat from above may be also employed, for instance by means of hot non-oxidizing combustion gases streaming along above the layer of the zinc vapours produced from said bath.

The process may be carried into effect in an oscillating kiln of preferably drum-like shape too, in connection therewith, however, care must be taken to prevent that the melting-bath should be mixed by said oscillation of the kiln so violently as to render the separation of the metallic impurities by eliquation and deposition impossible. Furthermore, the process may be effected in a stationary kiln too having the form of a channel or duct and being fitted with any kind of a bottom heating, the said bottom being provided with a pocket-like depression exempted in as great a degree as possible from the effect of said bottom heating. In this case also the combustion of the zinc vapours may be effected either above the smelting-bath or in a separate combustion chamber.

In all variations of the invention a stream of reducing gases (for instance CO) or other non-oxidizing i. e. neutral gases may be employed if desired for removing the zinc vapours from the evaporation chamber  $a_4$  and for transporting them into the special combustion chamber  $g$ .

The alternate introduction of a stream of reducing or other non-oxidizing gases offers substantial advantages in connection with that variety of the process according to the invention

in which the combustion of the zinc vapours takes place in the evaporation chamber  $a_4$  itself in order to utilize the heat of combustion of the zinc from above as radiated heat and possibly also as bottom heating by having the kiln rotated and/or oscillated. In connection therewith I have noticed that the said heat of combustion if it acts continuously without interruption may cause overheating, and in consequence thereof the metal bath may get into a condition of violent boiling, or may show a tendency towards the formation of bubbles whereby as has already been mentioned previously the process of separating the impurities by elutriation and/or deposition is affected disadvantageously. In order to avoid the said overheating it is advisable to introduce alternately a stream of gases of oxidizing nature (for instance air and/or  $\text{CO}_2$ ) and then gases of a reducing or other non-oxidizing nature (for instance  $\text{CO}$ ). Thereby the bottom heating of the metal bath is cut out temporarily and during the periods of introduction of said neutral or reducing gases an opportunity is offered to the metal bath for giving off any surplus heat content which may have been taken up by it during the time when oxidizing gases are streaming above the layer of zinc vapours produced. The length of time of said alternations has to be suited to the conditions of operation and depends on the degree of purity of the initial materials employed in each case. In a given case the stream of oxidizing gases may be cut out each time after a period of about 4 hours in order to replace it by a stream of neutral and/or reducing gases for a period of about 15 minutes. By using the non-oxidizing gases for removing the zinc vapours from chamber  $a_4$  and transporting them into special combustion chamber  $g$ , continuity in the production of zinc white may be ensured.

The gases of a reducing or other non-oxidizing nature which are applied intermediately or intermittently are admitted to the evaporation chamber  $a_4$  preferably in a heated condition in order to avoid any too rapid cooling-down in the evaporation chamber. The said gases may be taken from a gas generator inserted in series directly before the evaporation chamber  $a_4$  so that the own inherent heat of said gases may be utilized too.

The temporary replacement of the oxidizing atmosphere by a neutral and/or reducing atmosphere also offers advantages and may be employed according to the invention even in cases

when the separation of the impurities is effected according to the previously mentioned processes of the inventor because the boiling and bubbling of the bath always impairs the said separation of the impurities.

What I claim is:

1. A method of manufacturing zinc white pigments which consists in melting in a chamber a metal containing zinc and impurities such as lead, passing a stream of oxidizing gas through the chamber above the surface of the molten metal to oxidize the zinc vapors generated from said molten metal and heating the bath in the chamber from above by means of the radiated heat produced by said oxidation to generate further zinc vapors, periodically interrupting the oxidation by eliminating the passage of the oxidizing gas and substituting therefor a stream of non-oxidizing gas above the molten metal to thereby reduce the temperature of the bath to a degree to prevent a violent boiling and bubbling of the bath, the zinc vapors generated during the flow of non-oxidizing gases being transferred by said flow into a separate chamber where they are oxidized.

2. A method of manufacturing zinc white pigments which consists in melting in a chamber having the form of a rotating drum a metal bath containing zinc and impurities such as lead, passing an oxidizing gas in a stream above the surface of the molten metal to oxidize the zinc vapors generated from said metal while at the same time heating the metal by means of the heat produced by said oxidation in heating the wall of the drum, the rotation of the drum utilizing the heat of the oxidation throughout the wall of the drum for heating the metal, interrupting the passage of the oxidizing gas at predetermined periods and substituting therefor a stream of non-oxidizing gas to thus materially reduce the heat of the wall of the revolving drum and of the metal to avoid that violent boiling and bubbling of the bath which would tend to vaporize impurities in the bath for mingling with the zinc vapor, and transferring the zinc vapors moved under the influence of the non-oxidizing gas to an oxidizing chamber located beyond the drum.

3. A method as defined in claim 2, wherein the passage of the non-oxidizing gases takes place at intervals of approximately three hours and is maintained for periods approximating twenty minutes.

CORNELIUS RAYMOND BINGER.